

## UNITED STATES PATENT OFFICE

2,448,605

COMPOSITION FOR TREATING COAL  
AND THE LIKEWerner E. Kleinicke, Manhasset, N. Y., assignor  
to The Johnson-March Corporation, New York,  
N. Y., a corporation of DelawareNo Drawing. Application November 13, 1944,  
Serial No. 563,321

6 Claims. (Cl. 106—123)

1

This invention relates to a novel composition adaptable for use in the treating of coal, coke, and the like, more particularly for allaying and preventing dusting of coal, coke, and the like.

Heretofore, as is well known, coal has been treated by spraying with petroleum oil to allay dust. Such treatment has been found useful, but is subject to substantial limitation in that it is not substantially effective in the treatment of damp and wet or washed coal due to the immiscibility of water and oil, which prevents the oil from adhering to the surface of the coal and permits the enlargement of globules deposited on the wet surface to droplets, the majority of which drain off the coal with the excess washing water.

Again, it has been found that for effective treatment the cheaper grades of fuel oil, such, for example, as Bunker C, are not effective for use because of their lack of spreadability.

Various efforts have been made to utilize the cheaper grades of fuel oil, such as Bunker C, for the treatment of coal, but it has been found that even preheating and extreme atomization did not effectively promote the spreading of such oils into the required thin continuous film over the coal particles to render the coal acceptably dustless.

Now in accordance with this invention, there is provided a composition which when added to petroleum oil of the types heretofore used or to the cheaper grades of fuel oil such as Bunker C, will insure the formation of a desired thin, adherent film of oil over the particles of the coal and render the coal desirably dustless. In the alternative, the ingredients of the composition according to this invention may be added separately to petroleum oil to be sprayed on coal with like effect to that obtained by addition of the composition to the oil.

The composition in accordance with this invention will contain essentially an unsaturated fatty acid having 18 carbon atoms, or a mixture of such acids, with which will desirably also be included an oil-soluble wetting agent.

The unsaturated fatty acid having 18 carbon atoms may, for example, be oleic acid, linoleic acid, or the like, or may, and desirably will, comprise tall oil which, as is well known, is a by-product of the sulfite pulp process and contains a large percentage of oleic and linoleic acids, and in addition rosin acids and sterols. A petroleum oil miscible solvent for the tall oil is desirably also included in the composition, though it will be understood that a petroleum oil miscible solvent

2

will desirably be included even where a fatty acid, or mixtures of fatty acids as such, are used rather than tall oil. Where a wetting agent is included the solvent will be such as to also dissolve the wetting agent.

The wetting agent will be soluble in petroleum oil and, for example, may be aryl alkyl polyether alcohol, such, for example, as is marketed by Rohm & Haas, under the name Triton NE, a highly sulfonated alkyl aryl compound, such, for example, as is marketed by Arnold, Hoffman & Co., under the name Ahcowet ANS, an ester of a sulfodicarboxylic acid, such as sodium dioctyl sulfosuccinate, marketed under the name Aerosol OT by Cyanamid Co.

Where a solvent is included in the composition, as will be especially desirable where tall oil is used in order to prevent crystallizing out of the rosin acids, the solvent may be any liquid which will dissolve the unsaturated fatty acids or tall oil and the wetting agent and which will be at the same time miscible with the petroleum oil to be sprayed on the coal.

By way of example and illustration, the solvent will desirably have a low pour test and low viscosity. The solvent may, for example, be a petroleum derivative, preferably a light petroleum oil, a coal tar derivative, a wood distillation product, or the like, boiling within the range 350-650° F. and desirably will have a high aromatics content, for example, 75% or more. By way of specific example, a suitable solvent, comprises a petroleum derivative boiling within about the range 350-650° F., having a pour test °F. of -40° F., a Saybolt Universal viscosity at 100° F. of 30-40, containing a minimum of about 75% aromatics and a maximum of about 15% olefin. Such product is presently marketed by Sun Oil Company under the name Sun 151-B.

With reference to the solvent, it will be understood, however, that the solvent may comprise oil of the type to be sprayed upon coal.

As has been indicated, an unsaturated fatty acid having 18 carbon atoms, or a mixture of such acids and, where included, an oil-soluble wetting agent may be added, either in admixture or separately, directly to the oil to be sprayed on the coal. In such case the oil to be sprayed will serve as a solvent for the fatty acid, or fatty acids, or the tall oil, where such is used, as well as for the wetting agent where such is included.

On the other hand, the fatty acid, or mixture of fatty acids, or tall oil and the wetting agent, where included, may be combined for shipment for addition to oil to be sprayed on coal at a dis-

tant point. Such composition, for example, may contain from 80 to 99.8 parts by weight of fatty acid to 0.2 to 20 parts by weight of oil soluble wetting agent. Such compositions may be added to oil to be sprayed on coal in amount within about the range 3 to 20 parts by weight of the said composition to 80 to 97 parts by weight of oil. As a more specific illustration, a suitable composition may be made up on the following formula:

## Formula No. 1

Pounds

|                                             |    |
|---------------------------------------------|----|
| Tall oil                                    | 95 |
| An alkyl aryl polyether alcohol (Triton NE) | 5  |

The composition according to the above formula may be efficiently added to, for example, Bunker C oil on the basis of 3 pounds of the above composition to 97 pounds of Bunker C oil. It being appreciated that while the composition according to the above formula will desirably be made up and shipped to the point of use of the oil and then mixed with the oil, the ingredients of the composition may be separately added to and admixed with the oil at the point of use or at the source of the oil.

As illustrative of compositions in accordance with this invention including a solvent, for example, to the composition according to the No. 1 formula may be added 10 pounds of a light petroleum coal tar or wood distillate, preferably one containing a substantial amount of aromatics. Again, by way of more specific example, compositions including a solvent may be made up on the following formulae:

## Formula No. 2

Pounds

|                      |    |
|----------------------|----|
| Tall oil             | 85 |
| Petroleum derivative | 15 |

## Formula No. 3

Per cent by weight

|                                                                                          |      |
|------------------------------------------------------------------------------------------|------|
| Tall oil                                                                                 | 50   |
| An alkyl aryl polyether alcohol (Triton NE)                                              | 0.2  |
| Petroleum derivative boiling 350-650° F. and containing a minimum of about 75% aromatics | 48.8 |

About 5% by weight of the composition according to Formula No. 2 may be added to, for example, Bunker C oil for spraying on coal, while about 5% by weight of the composition according to Formula No. 3 may be efficiently added to, for example, Bunker C oil for spraying on coal.

It will now be appreciated that the addition of composition in accordance with this invention to be sprayed on coal will greatly increase the spreadability of the oil when sprayed on wet or washed coal and will cause the oil to spread out upon the particles of coal with substantially uniform distribution in the form of a thin film.

Again, the addition of compositions in accordance with this invention to the cheaper grades of oils, such as Diesel oil, Bunker C oil, and the like, heretofore not usable, will greatly promote the spreadability of such oils when applied to wet or washed coal and render them effective for the dustproofing of such coal.

The addition of compositions according to the above formulae to oils applied to wet or washed coal will, as will now be appreciated, greatly increase the spreadability of the oils, and particularly in the case of Bunker C oil, heretofore not

effectively usable, thus enabling a very substantial increase in the amount of coal which can be effectively treated with a given amount of oil.

It will now be understood that this invention 5 contemplates primarily an additive for petroleum oil to be sprayed on coal to render it dustless. However, it will be understood that the composition formed by the addition to oil to be sprayed on coal of the components of the additive separately or in partial combination, is contemplated 10 as the full equivalent of the additive.

What I claim and desire to protect by Letters Patent is:

1. A composition according to claim 5, characterized by the fact that tall oil comprises the fatty acid.

2. A composition according to claim 5, characterized by the fact that a petroleum derivative boiling within about the range 350-650 F. and containing a minimum of about 75% aromatics comprises the petroleum oil miscible solvent.

3. A composition according to claim 5, characterized by the fact that an alkyl aryl polyether alcohol comprises the petroleum oil soluble wetting agent.

4. A composition according to claim 5, characterized by the fact that tall oil comprises the fatty acid, an alkyl aryl polyether alcohol comprises the petroleum oil soluble wetting agent and a petroleum derivative boiling within the range 350-650° F. and containing a minimum of about 75% aromatics comprises the petroleum oil miscible solvent.

5. A composition for application to coal to allay dusting comprising, in admixture, an unsaturated fatty acid having 18 carbon atoms, a petroleum oil soluble wetting agent, a low viscosity hydrocarbon distillate having a high aromatic component solvent for the said acid and wetting agent and miscible with petroleum oil and in dominating proportion a petroleum oil of the order of Bunker C oil.

6. A composition according to claim 5, characterized by the fact that the unsaturated fatty acid is in amount within about the range 80-99.8 parts by weight, that the petroleum oil soluble wetting agent is in amount within about the range 0.2-20 parts by weight and that the oil miscible solvent for the fatty acid and wetting agent is a petroleum derivative boiling within about the range 350-650° F. and contains a minimum of about 75% aromatics.

WERNER E. KLEINICKE.

## REFERENCES CITED

The following references are of record in the file of this patent:

## UNITED STATES PATENTS

| 60 | Number    | Name         | Date          |
|----|-----------|--------------|---------------|
|    | 1,621,483 | Dimmig       | Mar. 15, 1927 |
|    | 1,903,879 | Rheiner      | Apr. 18, 1933 |
|    | 1,919,125 | Patch et al. | July 18, 1933 |
|    | 1,988,999 | Cunningham   | Jan. 22, 1935 |
| 65 | 2,157,294 | Lier         | May 9, 1939   |
|    | 2,222,370 | Mori         | Nov. 19, 1940 |
|    | 2,326,120 | Black        | Aug. 10, 1943 |
|    | 2,349,044 | Jahn         | May 16, 1944  |

## OTHER REFERENCES

"Practical Emulsions," Bennett (1943), page 107.